



US006521400B1

(12) **United States Patent**  
Dannhauser et al.

(10) **Patent No.:** US 6,521,400 B1  
(45) **Date of Patent:** Feb. 18, 2003

(54) **IMAGE MODIFICATION IN COLOR  
REVERSAL PHOTOGRAPHIC ELEMENTS**

(75) Inventors: **Thomas J. Dannhauser**, Pittsford, NY (US); **Phillip D. Knight**, Fairport, NY (US); **Thomas R. Welter**, Webster, NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/590,483**

(22) Filed: **Jun. 8, 2000**

(51) Int. Cl.<sup>7</sup> ..... **G03C 1/34**

(52) U.S. Cl. ..... **430/544; 430/547**

(58) Field of Search ..... 430/544, 547

(56) **References Cited**

U.S. PATENT DOCUMENTS

|               |         |                   |       |         |
|---------------|---------|-------------------|-------|---------|
| 3,536,487 A   | 10/1970 | Graham            | ..... | 430/504 |
| 3,674,478 A   | 7/1972  | Grasshoff et al.  | ..... | 430/219 |
| 3,730,724 A   | 5/1973  | Abbott            | ..... | 430/505 |
| 4,248,962 A   | 2/1981  | Lau               | ..... | 430/382 |
| 4,350,752 A   | 9/1982  | Reczek et al.     | ..... | 430/219 |
| 4,478,929 A   | 10/1984 | Jones et al.      | ..... | 430/217 |
| 4,684,604 A   | 8/1987  | Harder            | ..... | 430/375 |
| 4,845,020 A   | 7/1989  | Itoh et al.       | ..... | 430/445 |
| 4,861,701 A * | 8/1989  | Burns et al.      | ..... | 430/543 |
| 5,019,492 A   | 5/1991  | Buchanan et al.   | ..... | 430/543 |
| 5,041,367 A   | 8/1991  | Sniadoch          | ..... | 430/603 |
| 5,116,717 A   | 5/1992  | Matsushita et al. | ..... | 430/264 |
| 5,380,633 A   | 1/1995  | Harder et al.     | ..... | 430/505 |
| 5,411,839 A   | 5/1995  | Harder et al.     | ..... | 430/379 |
| 5,567,577 A   | 10/1996 | Welter et al.     | ..... | 430/544 |

FOREIGN PATENT DOCUMENTS

|    |            |         |
|----|------------|---------|
| EP | 255 085    | 2/1988  |
| JP | 4 040 450  | 2/1992  |
| JP | 7 311 433  | 11/1995 |
| JP | 7 311 437  | 11/1995 |
| JP | 10 282 616 | 10/1998 |
| JP | 11 327 102 | 11/1999 |

OTHER PUBLICATIONS

U.S. patent application Ser. No. 09/060,802, filed Apr. 15, 1998, titled "Photographic Elements Containing Release Compounds", of Vargas et al.

\* cited by examiner

Primary Examiner—Hoa Van Le

(74) Attorney, Agent, or Firm—Andrew J. Anderson

(57)

ABSTRACT

A multilayer color reversal photographic film element is described containing at least two silver halide photographic emulsion layers and a compound of the formula F-1:

F-1



wherein A, B, C, and D are independently substituted or unsubstituted aliphatic, alicyclic, aromatic or heterocyclic substituents, which may where structurally possible together form a ring or rings; where at least one of A, B, C, and D is of the formula F-2:

F-2



wherein R<sup>1</sup> and R<sup>2</sup> are independently either hydrogen or substituted or unsubstituted aliphatic, alicyclic, aromatic or heterocyclic substituents, which may where structurally possible form a ring with other substituents; R<sup>3</sup> is a substituted or unsubstituted aliphatic, alicyclic, aromatic or heterocyclic substituent which may where structurally possible form a ring with other substituents, L is a bivalent linking or timing group attached to the carbonyl moiety via a heteroatom, n varies from 0–2; and INH is a silver development inhibitor attached either to an L or the carbonyl moiety via a heteroatom.

**20 Claims, No Drawings**

# IMAGE MODIFICATION IN COLOR REVERSAL PHOTOGRAPHIC ELEMENTS

## FIELD OF THE INVENTION

This invention relates to silver halide photographic elements. In particular, it relates to color reversal photographic elements containing release compounds which provide a non-imagewise distribution of an image-modifying compound.

## BACKGROUND OF THE INVENTION

Conventional color photographic images are formed via a chromogenic development process comprising reaction of oxidized silver halide developing agent and dye precursors known as color couplers. After exposure of a color photographic element, the object scene is typically stored as a composite of red, green and blue latent silver halide images. During processing, these images or related reversal silver halide images are reductively developed in presence of a phenylenediamine color developer. Oxidized developer produced under these conditions reacts with the conjugate base of cyan, magenta or yellow dye-forming couplers to give their respective dyes. The composite dye image is then formed by the superpositioning of the cyan, magenta and yellow dye images to afford a reproduction of the original scene.

Color reproduction and image sharpness are important features of photographic reproductions. The color reproduction of conventional photographic system is primarily controlled by the hues of the cyan, magenta and yellow dyes that comprise the color image. Such image dyes, while generally reproducing a wide range of colors accurately, are never ideal; imperfections in the spectral characteristics of these dyes lead to degraded color reproduction. Thus, a yellow dye that absorbs too much green light appears orange and cannot effectively reproduce bright yellows, e.g. lemons. This yellow dye in combination with an effective magenta dye affords desaturated red colors, e.g. flowers or textiles.

In forming photographic images, it has become relatively common practice in the art to incorporate image-modifying compounds into either the developing solutions or the photographic materials themselves. These image-modifying compounds can impact such photographic properties as sharpness, granularity, contrast and color reproduction. Major changes in color reproduction can be obtained via alterations in the chemical nature of the image dye couplers, but a more subtle color correction mechanism is often employed: interlayer interimage effects (IIE). IIE occurs when the development process of one color record changes that of one or more of the other records. The most typical application of IIE for color correction is to inhibit the formation of one dye in response to the formation of another. In the case of the de-saturated red colors mentioned above, the imperfect yellow dye absorbs some green light, thus, less than a theoretical amount of magenta dye is needed for adequate red color reproduction. During the design of modern films, mechanisms for such IIE's have been perfected. Most typically a development inhibitor, perhaps iodide from the emulsion or an organic development inhibitor derived from a development inhibitor releasing (DIR) coupler, are produced in one layer (the causing layer); this inhibitor, upon migration to another imaging layer (the receiver layer), suppresses development to eventually yield the desired color reproduction effect.

Negative materials are processed, after image exposure, directly with a chromogenic developer which color-develops

the negative exposed areas. Positive dye image-forming reversal photographic materials, on the other hand, after imagewise exposure, are first processed with a black-and-white developer which develops a silver image in the negative exposed areas. This is followed by a reversal fogging step (e.g., a second overall exposure or a chemical fogging step) and then development with a chromogenic developer to form a positive color image. In negative dye image-forming photographic materials, interimage effects are always obtained during chromogenic development. In positive dye image-forming reversal photographic materials, interimage effects are generally obtained during processing by the release in the first black-and-white developer of a development inhibitor as a function of the silver development of the image-forming layers. The most generally used development inhibitor consists of iodide ions released as a result of the development of silver haloiodide, for example, silver bromoiodide emulsions.

In some color reversal films IIE's derived from inhibition in the black-and-white development step can be amplified via the inclusion of certain chemical addenda; often 4-carboxymethyl-2-mercaptopthiazole (CMMT, CAS #36365-79-4) or related compounds are employed in this manner.



Frequently the beneficial effects of the presence of silver development inhibitors comes with a loss in photographic speed, due to losses incurred during the inhibition of emulsion development or via the interaction of the coated inhibitor with the photographic emulsion. The inclusion of CMMT or similar development inhibitors in color reversal films improves the color reproduction and sharpness of the image but with a substantial speed penalty. Direct incorporation of image-modifying compounds into photographic materials also often leads to unacceptable image reproduction as such compounds can prematurely interact with other components of the photographic elements, or can decompose during shelf keeping. Thus, methods for the incorporation of development inhibitors into photographic films that circumvent these disadvantage are of particular interest.

It has become accepted to attach image-modifying compounds to coupler moieties and to have them released in an imagewise manner during development of the photographic material. This, however, has the dual disadvantage of requiring image formation (as the coupler moiety reacts with oxidized developer) whenever the presence of an image-modifying compound is desired, and of providing only an imagewise release of the image-modifying compound. Materials that afford imagewise delivery of inhibitors during reversal black and white development, often termed inhibitor releasing developers (IRD's), have also been described previously (e.g. U.S. Pat. Nos. 4,636,456, 5,210,012, 5,310, 638, 5,541,044, 5,578,441, and 5,756,274; JP Kokai 11-327102). While potentially providing valuable photographic improvements, the useful embodiments of this technology are disadvantageous in two regards. Firstly, these compounds are oxidatively unstable, shortening product shelf life. Aerial oxidation of IRD's, during film storage, can initiate a chain of reactions leading to the premature release of development inhibitor that degrades photographic behav-

ior. This is similar to the disadvantage of direct incorporation of development inhibitors describe above. Secondly, the imagewise delivery of the inhibitor by oxidative consumption of the IRD during development, by its very mechanism, necessitates the presence of residual IRD in the film after development. This residue when carried into the color developer can itself afford two disadvantages. First, the IRD can reductively consumed oxidized color developer leading to reduced image dye formation. In the second place, the residual IRD now provides delivery of a development inhibitor during the color development step; this release can limit or slow chromogenic development perhaps leading to reduced image dye formation or to an increased sensitivity of the film to processing solution variability.

There are known alternative means for incorporating image-modifying compounds into various types of photographic materials. Image modifying compounds have been inactivated by blocking as disclosed in, for example, U.S. Pat Nos. 3,674,478, 4,350,752, 4,478,929, 4,684,604, 5,019, 492, 5,116,717, and 5,567,577; EP 0 255 085; and JP Kokai 7-311437. Although some of the blocked or timed inhibitors known in the art are capable of impacting photographic properties primarily during the initial black and white development step of reversal processing, at certain levels or in certain photographic elements, the may be inadequate for completely controlling color balance. While the use of certain quinone based blocked inhibitor compounds is conventional in dye image transfer film systems as disclosed, e.g., in U.S. Pat. No. 4,478,929, there is no suggestion such compounds may be advantageously used in color reversal materials. Similarly, While JP Kokai 7-311437 suggests the use of development inhibitor releasing quinone compounds in a graphic arts silver halide product, there is no suggestion such compounds may be advantageously used in color reversal materials.

#### SUMMARY OF THE INVENTION

It is an object of the present invention to provide color reversal photographic materials comprising blocked image-modifying compounds that are unblocked in a non-imagewise manner and that provide adequate control over image modification.

In accordance with one embodiment of the invention, a multilayer color reversal photographic film element is described containing at least two silver halide photographic emulsion layers and a compound of the formula F-1:



wherein A, B, C, and D are independently substituted or unsubstituted aliphatic, alicyclic, aromatic or heterocyclic substituents, which may where structurally possible together form a ring or rings; where at least one of A, B, C, and D is of the formula F-2:



10 wherein R<sup>1</sup> and R<sup>2</sup> are independently either hydrogen or substituted or unsubstituted aliphatic, alicyclic, aromatic or heterocyclic substituents, which may where structurally possible form a ring with other substituents; R<sup>3</sup> is a substituted or unsubstituted aliphatic, alicyclic, aromatic or heterocyclic substituent which may where structurally possible form a ring with other substituents, L is a bivalent linking or timing group attached to the carbonyl moiety via a heteroatom; n varies from 0-2; and INH is a silver development inhibitor attached either to an L or the carbonyl moiety via a heteroatom. In preferred embodiments, R<sup>1</sup> and R<sup>2</sup> are hydrogen or lower alkyl groups of from 1 to 4 carbon atoms, R<sup>3</sup> is an alkyl group (more preferably primary alkyl group) of from 1-12 carbon atoms, and A, B, C and D substituents which are not of structure F-2 are preferably alkyl or aryl groups of from 1-20 carbon atoms. A second embodiment of the invention comprises subjecting a color reversal film as described above after imagewise exposure to a color reversal process comprising a first black and white development step which develops a silver image in negative exposed areas, a reversal fogging step, and then development with a chromogenic developer to form a positive color image.

20 It has been found that use of the benzoquinone derivatives of Formula F-1, capable of redox-derived release of development inhibitors, can afford improved acutance and color 30 of reversal films. These improvements resulting from the use of inhibitor releasing quinone (IRQ) compounds come at a lower speed penalty than that from the directly incorporated development inhibitor, and provide an alternative mechanism by which development inhibitors can be released in a non-imagewise manner during color reversal processing. Potential problems related to the use of IRD's are also 40 circumvented. The IRQ compound incorporates the development inhibitor into the film as an oxidized substrate with good shelf life, particularly with regard to aerial oxidation. 45 The non-imagewise delivery of inhibitors from this technology during black and white development is not mechanically constrained to leave residual amounts of unconsumed masked inhibitor remaining in the film.

#### DETAILED DESCRIPTION OF THE PREFERRED EMBODIMENTS

Photographic film elements in accordance with the invention contain a compound of the formula F-1:



55 60 65 wherein A, B, C, and D are independently substituted or unsubstituted aliphatic, alicyclic, aromatic or heterocyclic substituents, which may where structurally possible together

form a ring or rings; wherein at least one of A, B, C, and D is of the formula F-2:

F-2  
5

10

wherein R<sup>1</sup> and R<sup>2</sup> are independently either hydrogen or substituted or unsubstituted aliphatic, alicyclic, aromatic or heterocyclic substituents, which may where structurally possible form a ring with other substituents; R<sup>3</sup> is a substituted or unsubstituted aliphatic, alicyclic, aromatic or heterocyclic substituent which may where structurally possible form a ring with other substituents, L is a bivalent linking or timing group attached to the carbonyl moiety via a heteroatom; n varies from 0-2; and INH is a silver development inhibitor attached either to an L or the carbonyl moiety via a heteroatom.

Representative aliphatic, alicyclic, aromatic or heterocyclic substituents for groups A, B, C, D, R<sup>1</sup>, R<sup>2</sup>, and R<sup>3</sup> include primary, secondary, and tertiary alkyl groups, cycloalkyl groups such as cyclopentyl and cyclohexyl, phenyl and naphthyl groups, and heterocyclic groups such as pyridyl, furanyl, pyrrolyl, piperidinyl. In preferred embodiments, R<sup>1</sup> and R<sup>2</sup> are hydrogen or lower alkyl groups of from 1 to 4 carbon atoms, R<sup>3</sup> is an alkyl group (more preferably primary alkyl group) of from 1-12 carbon atoms, and A, B, C and D substituents which are not of structure F-2 are preferably alkyl or aryl groups of from 1-20 carbon atoms.

L is a linking or timing group that, upon activation or timing, is capable of releasing the INH. Such timing groups are well known in the art, and representative timing groups are as described, e.g., in Research Disclosure No. 36544 (1994) pg. 525 and U.S. Pat. No. 5,474,886, the disclosures of which are incorporated herein by reference.

INH is a releasable inhibitor compound. When incorporated in the inhibit or releasing quinone compound F-1 in a deactivated form, such compounds provide both good shelf life and controlled release into developing emulsion, via chemical interaction between the F-1 compound and a reductive developer bath. INH compounds may include any of a variety of known development inhibitors, such as are described in such representative patents as U.S. Pat. No. 3,227,554; U.S. Pat. No. 3,384,657; U.S. Pat. No. 3,615,506; U.S. Pat. No. 3,617,291, U.S. Pat. No. 3,733,201 and U.K. Patent 1,450,479 (also see T. H. James, in *The Theory of the Photographic Process*, 4th Ed., Macmillan, New York, 1977, chapter 13J; and *Research Disclosure*, December 1989, Item No. 308911, Section VI and references therein). Preferred INH compounds are heterocyclic compounds such as mercaptotetrazoles, selenotetrazoles, mercaptobenzothiazoles, selenobenzothiazoles, mercaptobenzoxazoles, selenobenzoxazoles, benzotriazoles, and benzodiazoles, mercaptooxadiazoles, mercaptothiadiazoles, and mercaptothiazoles. General structures of preferred development inhibitors INH include:

INH-1



INH-2



INH-3



INH-4



INH-5



INH-6



INH-7



INH-8



INH-9



INH-10



where R<sup>7</sup> and R<sup>8</sup> are individually hydrogen, a substituted or unsubstituted alkyl (preferably of 1 to 8 carbon atoms, for example, methyl, ethyl, butyl) or phenyl group, and R<sup>9</sup> and R<sup>10</sup> are individually hydrogen or one or more halogen (for example, chloro, fluoro, bromo), alkyl (preferably of 1 to 4 carbon atoms), carboxyl, carboxy esters (such as —COOCH<sub>3</sub>), —NHCOOCH<sub>3</sub>, —SO<sub>2</sub>OCH<sub>3</sub>, —OCH<sub>2</sub>CH<sub>2</sub>SO<sub>2</sub>CH<sub>3</sub>, —OC(O)OCH<sub>2</sub>CH<sub>3</sub>, —NHC(O)C(O)OCH<sub>3</sub> or nitro groups.

In a particular embodiment, presence of a solubilization group having a low pKa (e.g., less than 10, more preferably less than 7) facilitates reductive release of the inhibitors. Useful examples of acidic functional groups or salts thereof with an aqueous pKa of less than 10 include carboxylic acids, carboxylic salts, sulfonic acids, sulfonic acids,

cyanamides, sulfonamides, hydroxamic acids, thiols, thiolates, and the like. Most suitable are carboxylic acids, carboxylate salts, and sulfonic acids. The site of this solubilization could be on substituents A, B, C or D which are not F-2, on the F-2 substituents (e.g., the R<sup>1</sup>, R<sup>2</sup>, R<sup>3</sup> or L groups), or on the INH. In the most preferred embodiments of the invention, the solubilization group, when present, is on either an A, B, C or D substituent or the INH in the form of a carboxylic acid moiety.

Mercaptothiazoles such as CMMT and its lower esters are especially preferred as INH groups for F-1 compounds in accordance with the invention, i.e. where INH is of the structure:



where R<sub>i</sub> is hydrogen or alkyl group of from 1-4 carbon atoms.

Where only one of the A, B, C, D substituents is of the structure F-2 (i.e., a mono INH-releasing quinone), a particularly preferred embodiment is where the meta and para positioned substituents (relative to the F-2 substituent) form a carbocyclic ring (most preferably a non-aromatic ring) and the ortho positioned substituent is a primary, secondary, or tertiary alkyl group, and the R<sup>3</sup> group of the F-2 substituent is a primary alkyl group.

Where two of the A, B, C, D substituents are of the structure F-2 (i.e., a bis INH-releasing quinone), they may be positioned ortho, meta, or para with respect to each other, but para positioning is preferred for ease of synthesis. The remaining A, B, C, D substituents preferably are primary, secondary, or tertiary alkyl groups, and the R<sup>3</sup> groups of the two F-2 substituents are preferably primary alkyl groups.

The presence of three or four F-2 groups is specifically contemplated, but less preferable for synthesis purposes.

The blocked image-modifying compounds of the present invention provide for the opportunity to specifically control the strength and location of image modification. They are also useful when incorporated in oligomeric or other polymeric species. Further, when such compounds unblock to form development inhibitors, excellent control of push processing, control of fog development, and control of specific layer developability can be obtained. These three applications can be realized by controlling the release rates. To control push processing, steady release upon extended processing is desirable; for control of fog development, gradual release during keeping is desirable; and for control of specific layer developability, rapid release upon processing is desirable.

One application of this technology may be to improve the color balance of reversal films. The reagent may be designed to not substantially affect development during normal processing time, but would upon extended development times (such as for push processing) reduce intralayer developability so as to match the developability of the other layers. These materials are stable when coated and at keeping pH. However, upon first developer processing (i.e., black and white development step in a color reversal process) they react with developers to gradually release the inhibitor. At longer processing times (such as during push processing) more inhibitor is released. Such control can be with regard

to different color records, or with regard to different layers (for example, fast or slow) in the same color record. Further, the reduction of maximum density that typically occurs during push processing can be minimized.

Unless otherwise specifically stated, substituent groups which may be substituted on molecules herein include any groups, whether substituted or unsubstituted, which do not destroy properties necessary for photographic utility. When the term "group" is applied to the identification of a substituent containing a substitutable hydrogen, it is intended to encompass not only the substituent's unsubstituted form, but also its form further substituted with any group or groups as herein mentioned. Suitably, the group may be halogen or 5 may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as 10 alkyl, including straight or branched chain alkyl, such as methyl, trifluoromethyl, ethyl, t-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, sec-butoxy, hexyloxy, 15 2-ethylhexyloxy, tetradecyloxy, 2-(2,4-di-t-pentylphenoxy) ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, 20 benzamido, butyramido, tetradecanamido, alpha-(2,4-di-t-pentyl-phenoxy)acetamido, alpha-(2,4-di-t-pentylphenoxy) butyramido, alpha-(3-pentadecylphenoxy)-hexanamido, alpha-(4hydroxy-3-t-butylphenoxy)-tetradecanamido, 2-oxo-pyrrolidin-1-yl, 2-oxo-5-tetradecylpyrrolin-1-yl, 25 N-methyltetradecanamido, N-succinimido, N-phthalimido, 2,5-dioxo-1-oxazolidinyl, 3-dodecyl-2,5-dioxo-1-imidazolyl, and N-acetyl-1-N-dodecylamino, ethoxycarbonylamino, phenoxy carbonylamino, benzoyxycarbonylamino, hexadecyloxycarbonylamino, 2,4-di-t-butylphenoxy carbonylamino, phenyl carbonylamino, 2,5-(di-t-pentylphenyl) carbonylamino, p-dodecylphenyl carbonylamino, p-tolyl carbonylamino, N-methylureido, N,N-dimethylureido, N-methyl-N-dodecylureido, N-hexadecylureido, N,N-dioctadecylureido, 30 N,N-dioctyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butylcarbonamido; sulfonamido, such as methylsulfonamido, benzenesulfonamido, 35 p-tolylsulfonamido, p-dodecylbenzenesulfonamido, N-methyltetradecylsulfonamido, N,N-dipropylsulfamoyl, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, 40 N-[4-(2,4-di-t-pentylphenoxy)butyl]sulfamoyl, N-methyl-N-tetradecylsulfamoyl, and N-dodecylsulfamoyl; carbamoyl, such as N-methylcaramoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-diethylcarbamoyl; acyl, such as acetyl, (2,4-di-t-aminophenoxy)acetyl, phenoxy carbonyl, p-dodecylphenoxy carbonyl, methoxycarbonyl, 45 butoxycarbonyl, tetradecyloxycarbonyl, ethoxycarbonyl, benzoyloxycarbonyl, 3-compounds of formula F-1 which may be employed in the present invention include IRQ-1 through IRQ-46 shown below:



-continued

IRQ-9



IRQ-10



IRQ-11



IRQ-12

IRQ-13



IRQ-14

IRQ-15



IRQ-16

IRQ-17





-continued

IRQ-18



IRQ-19



IRQ-20



IRQ-21



IRQ-22



IRQ-23



IRQ-24



IRQ-25



IRQ-26



IRQ-27



IRQ-28



IRQ-29

-continued

IRQ-30



IRQ-31



IRQ-32



IRQ-34



IRQ-35



IRQ-36



IRQ-37



IRQ-38



IRQ-39

IRQ-40



IRQ-41

IRQ-42



IRQ-43

-continued  
IRQ-44

IRQ-45

IRQ-46



Generally, the IRQ compounds employed in elements of this invention can be made using conventional synthesis techniques, as illustrated in the synthetic examples below.

The photographic elements of the present invention are multilayer color reversal photographic elements. Multicolor elements typically contain dye image-forming units sensitive to each of the three primary regions of the visible light spectrum. Each unit can be comprised of a single emulsion layer or of multiple emulsion layers sensitive to a given region of the spectrum. The layers of the element, including the layers of the image-forming units, can be arranged in various orders as known in the art. Dye-forming couplers may be incorporated into the emulsion layers, or may be introduced during processing (e.g., with standard published K-14 Kodachrome processing).

A typical coupler-incorporated multicolor photographic element comprises a support bearing a cyan dye image-forming unit comprising at least one red-sensitive silver halide emulsion layer having associated therewith at least one cyan dye-forming coupler; a magenta image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. Each silver halide emulsion unit can be composed of one or more layers and the various units and layers can be arranged in different locations with respect to one another. The element may contain additional layers, such as filter layers, interlayers, overcoat layers, subbing layers, and the like. The inhibitor releasing compounds of this invention can be incorporated in at least one of the silver halide emulsion layers and/or in at least one other layer, such as an adjacent layer. While it is an advantage of the invention that the use of inhibitor releasing quinone compounds of formula F-1 result in a lower speed penalty than that from conventional directly incorporated development inhibitors such as CMMT, such directly incor-

30

porated development inhibitors may be used in combination (in the same or different layers) with compounds of formula F-1 when desired.

Photographic emulsions are generally prepared by precipitating silver halide crystals in a colloidal matrix by methods conventional in the art. The colloid is typically a hydrophilic film forming agent such as gelatin, alginic acid, or derivatives thereof. The crystals formed in the precipitation step are washed and then chemically and spectrally sensitized by adding spectral sensitizing dyes and chemical sensitizers, and by providing a heating step during which the emulsion temperature is raised and maintained for a period of time. The precipitation and spectral and chemical sensitization methods utilized in preparing the emulsions employed in the invention can be those methods known in the art.

Chemical sensitization of the emulsion typically employs sensitizers such as: sulfur-containing compounds, e.g., allyl isothiocyanate, sodium thiosulfate and allyl thiourea; reducing agents, e.g., polyamines and stannous salts; noble metal compounds, e.g., gold, platinum; and polymeric agents, e.g., polyalkylene oxides. Preferably, the emulsion is sensitized both with gold and a chalcogenide, most preferably gold and sulfur. Examples of sulfur sensitizers include sodium thiosulfate, alkyl or aryl thiourea compounds, or thiourea compounds with nucleophilic substituents as described in U.S. Pat. No. 4,810,626. Examples of gold sensitizers include potassium tetrachloroaurate, potassium dithiocyanato gold(I), trisodium dithiosulfato gold(I), and the gold(I) compounds described in U.S. Pat. Nos. 5,049,484; 5,049,485; 5,252,455; 5,220,030; and 5,391,727. As described, heat treatment is employed to complete chemical sensitization. Spectral sensitization is effected with a combination of dyes, which are designed for the wavelength range of interest within the visible or infrared spectrum. It is known to add such dyes both before and after heat treatment.

After spectral sensitization, the emulsion is coated on a support. Various coating techniques include dip coating, air knife coating, bead coating, curtain coating and extrusion coating.

The compounds of this invention may be added to the silver halide emulsion at any time during the preparation of the emulsion, i.e., during precipitation, during or before chemical sensitization or during final melting and co-mixing of the emulsion and additives for coating. More preferably, these compounds are added during final melting and co-mixing of the emulsion and additives for coating.

Suitable levels of IRQ compounds of formula F-1 utilized in the present invention are about 0.02 to about 25 mmole/mole silver. Preferred levels are about 0.05 to about 15 mmole/mole silver. Most preferred levels are 0.1 to 2.0 mmole/mole silver.

The silver halide emulsion grains may be comprised of any halide combination, including silver chloride, silver bromide, silver bromochloride, silver chlorobromide, silver iodochloride, silver iodobromide, silver bromoiodochloride, silver chloroiodobromide, silver iodobromochloride, and silver iodochlorobromide emulsions. Preferred are iodobromide emulsions with an iodide content of 2 to 12%.

The emulsions employed in the elements of this invention can include silver halide grains of any conventional shape or size (e.g., cubical, octahedral, dodecahedral, spherical or tabular) of silver halide grains. Specifically, the emulsions can include coarse, medium or fine silver halide grains. It is preferred, however, that the present invention be practiced with tabular grains having an aspect ratio greater than 2:1, preferably at least 5:1, and optimally at least 7:1. Aspect ratio as used herein is understood to mean the ratio of the equivalent circular diameter of a grain to its thickness. The equivalent circular diameter of a grain is the diameter of a circle having an equal to the projected area of the grain. High aspect ratio tabular grain emulsions are specifically contemplated, such as those disclosed by Wilgus et al, U.S. Pat. No. 4,434,226, Daubendiek et al, U.S. Pat. No. 4,414,310, Wey, U.S. Pat. No. 4,399,215, Solberg et al, U.S. Pat. No. 4,433,048, Mignot, U.S. Pat. No. 4,386,156, Evans et al, U.S. Pat. No. 4,504,570, Maskasky, U.S. Pat. No. 4,400,463, Wey et al, U.S. Pat. No. 4,414,306, Maskasky, U.S. Pat. No. 4,435,501 and U.S. Pat. No. 4,643,966 and Daubendiek et al, U.S. Pat. No. 4,672 and U.S. Pat. No. 4,693,964, all of which are incorporated herein by reference. Also, specifically contemplated are those silver iodobromide grains with a higher molar proportion of iodide in the core of the grain than in the periphery of the grain, such as those described in British Reference No. 1,027,146; U.S. Pat. No. 4,379,837; U.S. Pat. No. 4,444,877; U.S. Pat. No. 4,665,012; U.S. Pat. No. 4,686,178 and U.S. Pat. No. 4,636,461 and in the European Reference No. 264,954, all of which incorporated herein by reference. The silver halide emulsions can be either monodisperse or polydisperse as precipitated. The grain size distribution of the emulsions can be controlled by silver halide grain separation techniques or be blending silver halide emulsions of differing grain sizes.

The grains can be contained in any conventional dispersing medium capable of being used in photographic emulsions. Specifically, it is contemplated that the dispersing medium be an aqueous gelatin-peptizer dispersing medium, of which gelatin—e.g., alkali treated gelatin (cattle bone and hide gelatin)—or acid treated gelatin (pigskin gelatin) and gelatin derivatives—e.g., acetylated gelatin, phthalated gelatin—are specifically contemplated. When used, gelatin is preferably at levels of 0.01 to 100 grams per total silver mole. Also contemplated are dispersing mediums comprised of synthetic colloids.

In the following Table, reference will be made to (1) Research Disclosure, December 1978, Item 17643, (2) Research Disclosure, December 1989, Item 308119, (3)

Research Disclosure, September 1994, Item 36544, and (4) Research Disclosure, September 1996, Item 38957, all published by Kenneth Mason Publications, Ltd., Dudley Annex, 12a North Street, Emsworth, Hampshire PO10 7DQ, ENGLAND, the disclosures of which are incorporated herein by reference. The Table and the references cited in the Table are to be read as describing particular components suitable for use in the elements of the invention. The Table and its cited references also describe suitable ways of preparing, exposing processing and manipulating the elements, and the images contained therein. Photographic elements and methods of processing such elements particularly suitable for use with this invention are described in Research Disclosure, February 1995, Item 37038, published by Kenneth Mason Publications, Ltd., Dudley Annex, 12a North Street, Emsworth, Hampshire PO10 7DQ, ENGLAND, the disclosure of which is incorporated herein by reference.

| Reference | Section                        | Subject Matter                                                                                    |
|-----------|--------------------------------|---------------------------------------------------------------------------------------------------|
| 1         | I, II                          | Grain composition, morphology and preparation.                                                    |
| 2         | I, II, IX, X, XI, XII, XIV, XV | Emulsion preparation including hardeners, coating aids, addenda, etc.                             |
| 25 3 & 4  | I, II, III, IX A & B           | Chemical sensitization and spectral sensitization/desensitization.                                |
| 1         | III, IV                        | UV dyes, optical brighteners, luminescent dyes.                                                   |
| 2         | III, IV                        | Antifoggants and stabilizers.                                                                     |
| 3 & 4     | IV, V                          |                                                                                                   |
| 1         | V                              |                                                                                                   |
| 30 2      | V                              |                                                                                                   |
| 3 & 4     | VI                             |                                                                                                   |
| 1         | VI                             |                                                                                                   |
| 2         | VI                             |                                                                                                   |
| 3 & 4     | VII                            |                                                                                                   |
| 1         | VIII                           | Absorbing and scattering materials, Antistatic layers, Matting agents.                            |
| 2         | VIII, XIII, XVI                |                                                                                                   |
| 35 3 & 4  | VIII, IX C & D                 | Image-couplers and image modifying couplers, Washout couplers, Dye stabilizers and hue modifiers. |
| 1         | VII                            | Supports                                                                                          |
| 2         | VII                            |                                                                                                   |
| 3 & 4     | X                              |                                                                                                   |
| 1         | XVII                           |                                                                                                   |
| 2         | XVII                           |                                                                                                   |
| 40 3 & 4  | XV                             | Specific layer arrangements.                                                                      |
| 3 & 4     | XI                             | Negative working emulsions;                                                                       |
| 3 & 4     | XII, XIII                      | Direct positive emulsions.                                                                        |
| 2         | XVIII                          | Exposure.                                                                                         |
| 1         | XIX, XX                        | Chemical processing;                                                                              |
| 2         | XIX, XX, XXII                  | Developing agents.                                                                                |
| 45 3 & 4  | XVIII, XIX, XX                 | Scanning and digital processing procedures.                                                       |
| 3 & 4     | XIV                            |                                                                                                   |

50 Supports for photographic elements of the present invention include polymeric films such as cellulose esters (for example, cellulose triacetate and diacetate) and polyesters of dibasic aromatic carboxylic acids with divalent alcohols (for example, poly(ethylene-terephthalate), poly(ethylene-naphthalates)). Such supports are described in further detail in Research Disclosure 3, Section XV. The photographic elements may also contain a transparent magnetic recording layer such as a layer containing magnetic particles on the underside of a transparent support. Magnetic layers have 55 been described in U.S. Pat. No. 4,279,945 and U.S. Pat. No. 4,302,523, and *Research Disclosure*, November 1992, Item No. 34390, which are incorporated herein by reference. Typically, the element will have a total thickness (excluding the support) of from about 5 to about 30 microns.

60 The photographic elements may also contain additional materials that accelerate or otherwise modify the processing steps of bleaching or fixing to improve the quality of the

image. Bleach accelerators described in European Patent Applications No. 193,389 and 301,477; U.S. Pat. Nos. 4,163,669; 4,865,956; and 4,923,784 are particularly useful. Also contemplated is the use of nucleating agents, development accelerators or their precursors (UK Patent 2,097,140; U.K. Patent 2,131,188); electron transfer agents (U.S. Pat. Nos. 4,859,578 and 4,912,025); antifogging and anti color-mixing agents such as derivatives of hydroquinones, aminophenols, amines, gallic acid; catechol; ascorbic acid; hydrazides; sulfonamidophenols; and non color-forming couplers.

The elements may also contain filter dye layers comprising colloidal silver sol and/or yellow and/or magenta filter dyes, either as oil-in-water dispersions, latex dispersions or as solid particle dispersions. Additionally, they may be used with "smearing" couplers (e.g. as described in U.S. Pat. No. 4,366,237; European Patent Application 96,570; U.S. Pat. No. 4,420,556; and 4,543,323.) Also, the couplers may be blocked or coated in protected form as described, for example, in Japanese Application 61/258,249 or U.S. Pat. No. 5,019,492.

The photographic elements may further contain other image-modifying compounds such as "Developer Inhibitor-Releasing" compounds (DIR's). IDIR compounds are disclosed, for example, in "Developer-Inhibitor-Releasing (DIR) Couplers for Color Photography," C. R. Barr, J. R. Thirtle and P. W. Vittum in Photographic Science and Engineering, Vol. 13, p. 174 (1969), incorporated herein by reference. DIRs that have particular application in color reversal elements are disclosed in U.S. Pat. Nos. 5,399,465; 5,380,633; 5,399,466; and 5,310,642.

The silver halide grains to be used in the invention may be prepared according to methods known in the art, such as those described in Research Disclosure 3 and James, The Theory of the Photographic Process. These include methods such as ammoniacal emulsion making, neutral or acidic emulsion making, and others known in the art. These methods generally involve mixing a water soluble silver salt with a water soluble halide salt in the presence of a protective colloid, and controlling the temperature, pAg, pH values, etc, at suitable values during formation of the silver halide by precipitation.

The silver halide to be used in the invention may be advantageously subjected to chemical sensitization with noble metal (for example, gold) sensitizers, middle chalcogen (for example, sulfur) sensitizers, reduction sensitizers and others known in the art. Compounds and techniques useful for chemical sensitization of silver halide are known in the art and described in Research Disclosure 3 and the references cited therein.

The emulsion can also include any of the addenda known to be useful in photographic emulsions. These include chemical sensitizers, such as active gelatin, sulfur, selenium, tellurium, gold, platinum, palladium, iridium, osmium, rhenium, phosphorous, or combinations thereof. Chemical sensitization is generally carried out at pAg levels of from 5 to 10, pH levels of from 5 to 8, and temperatures of from 30 to 80° C., as illustrated in Research Disclosure, June 1975, item 13452 and U.S. Pat. No. 3,772,031.

The silver halide may be sensitized by sensitizing dyes by any method known in the art, such as described in Research Disclosure 3. Examples of dyes include dyes from a variety of classes, including the polymethine dye class, which includes the cyanines, merocyanines, complex cyanines and merocyanines (i.e., tri-, tetra-, and poly-nuclear cyanines and merocyanines), oxonols, hemioxonols, stryryls, merostyryls, and streptocyanines. The dye may be added to

an emulsion of the silver halide grains and a hydrophilic colloid at any time prior to (e.g., during or after chemical sensitization) or simultaneous with the coating of the emulsion on a photographic element. The dye/silver halide emulsion may be mixed with a dispersion of color image-forming coupler immediately before coating or in advance of coating.

In a typical construction, a reversal film is distinguished from a color negative film in that it does not have any masking couplers. Furthermore, reversal films have a gamma generally between 1.5 and 2.0, a gamma which is much higher than the gamma for typical negative materials.

Photographic elements of the present invention can be imagewise exposed using any of the known techniques, including those described in Research Disclosure 3. This typically involves exposure to light in the visible region of the spectrum, and typically such exposure is of a live image through a lens. The photographic elements can be incorporated into exposure structures intended for repeated use or exposure structures intended for limited use, variously referred to as single use cameras, lens with film, or photo-sensitive material package units. However, the color reversal photographic elements of the present invention may alternatively be exposed in an electronic film writer. Exposure in a film writer is an exposure to a stored image (such as a computer stored image) by means of light emitting devices (such as light controlled by light valves, CRT, laser, laser diode, or some other controlled light source).

Silver halide color reversal films are typically associated with an indication for processing by a color reversal process. Reference to a film being associated with an indication for processing by a color reversal process, most typically means the film, its container, or packaging (which includes printed inserts provided with the film), will have an indication on it that the film should be processed by a color reversal process. The indication may, for example, be simply a printed statement stating that the film is a "reversal film" or that it should be processed by a color reversal process, or simply a reference to a known color reversal process such as "Process E-6" or "K-14". A "color reversal" process in this context is one employing a first developer treatment with a non-chromogenic developer (that is, a developer which will not imagewise produce color by reaction with other compounds in the film; sometimes referenced as a "black and white developer"). Black and white developing agents which may be used in the first development include dihydroxybenzenes or derivatives thereof, ascorbic acid or derivatives thereof, aminophenol and 3-pyrazolidone type developing agents. Such black and white developing agents are well known in the art, e.g., U.S. Pat. Nos. 5,187,050, 5,683,859, 5,702,875.

Preferred non-chromogenic developers are hydroquinones (such as hydroquinone sulphonate). The non-chromogenic development is followed by fogging unexposed silver halide, usually either chemically or by exposure to light. Then the element is treated with a color developer which will produce color in an imagewise manner upon reaction with other compounds (couplers), which may be incorporated in the film or introduced during processing. A wide variety of different color reversal processes are well known in the art. For example, a single color developing step can be used when the coupling agents are incorporated in the photographic element or three separate color developing steps can be used in which coupling agents are included in the developing solutions.

Preferred color developing agents are p-phenylenediamines. Especially preferred are: 4-amino N,N-diethylaniline hydrochloride; 4-amino-3-methyl-N,N-diethylaniline hydrochloride; 4-amino-3-methyl-N-ethyl-N-

25

(*b*-(methanesulfonamido)ethyl)aniline sesquisulfate hydrate; 4-amino-3-methyl-N-ethyl-*N*-(*b*-hydroxyethyl)aniline sulfate; 4-amino-3-*b*-(methanesulfonamido)ethyl-*N,N*-diethylaniline hydrochloride; and 4-amino-N-ethyl-N-(2-methoxyethyl)-*m*-toluidine di-*p*-toluene sulfonic acid.

Development is followed by bleach-fixing, to remove silver or silver halide, washing and drying. Bleaching and fixing can be performed with any of the materials known to be used for that purpose. Bleach baths generally comprise an aqueous solution of an oxidizing agent such as water soluble salts and complexes of iron (III) (e.g., potassium ferricyanide, ferric chloride, ammonium or potassium salts of ferric ethylenediaminetetraacetic acid), water-soluble per-

26

sulfates (e.g., potassium, sodium, or ammonium persulfate), water-soluble dichromates (e.g., potassium, sodium, and lithium dichromate), and the like. Fixing baths generally comprise an aqueous solution of compounds that form soluble salts with silver ions, such as sodium thiosulfate, ammonium thiosulfate, potassium thiocyanate, sodium thiocyanate, thiourea, and the like. Further details of bleach and fixing baths can be found in Research Disclosure 3. Standard commercial processing for reversal elements in accordance with the invention may preferably be utilized, including standard Kodak K-14 and Kodak E-6 processing.

## EXAMPLES

Synthetic Scheme for Preparation of IRQ-1:





-continued



Preparation of INT-1: A mechanically stirred slurry of naphthoquinone (CAS 130-15-4; 1.76 kg, 11.1 mole; Aldrich Chemical Co.) and 1,12-dodecanedioic acid (CAS 693-23-2; 2.30 kg, 10.0 mole; Fluka Chemie AG., pulverized pellets) in a mixture of 6.0 L water and 2.0 L acetonitrile was warmed to 75° C. (internal temperature) employing a steam bath. Silver nitrate (128 g, 0.75 mole; Acros Chemical Co.) catalyst was added in a single portion to the warm mixture. A solution of ammonium persulfate (3.42 kg, 15.0 mole; Aldrich Chemical Co.) in 4.4 L water (solution temperature warmed to 22° C. to complete dissolution) was added dropwise to the warm slurry over about 3 hours. Over the period of the addition, the temperature was maintained between 76–80° C. Very rapidly after the addition of the persulfate solution was begun, gas evolution (carbon dioxide) was noted; this gas evolution became vigorous as the reaction proceeded. After the completion of the addition, reaction mixture was stirred and the temperature maintained between 76–80° C. until gas evolution ceased, after 75 minutes. The mixture was cooled to just below ambient temperature and the solid filtered, washed with water (ca. 16 L in portions) and briefly air dried. The damp, crude solid was triturated with 8 L acetonitrile for about 30 minutes then filtered. The solids were washed with portions of acetonitrile (4×1 L), then air dried briefly. This damp crude material was dissolved in 6 L refluxing ethyl alcohol. The filtrate was allowed to cool slowly overnight, the resulting nearly solid mixture was mechanically dispersed, then filtered, pressed using a rubber dam then washed with minimal cold 3A alcohol (3×400 mL). Vacuum drying under a slow nitrogen steam afforded UNT-1 as a yellow solid (2.69 kg, 79%) mp 108–110° C.

Preparation of INT-2: A mechanically stirred slurry of INT-1 (513 g, 1.50 mole) in 1.50 L ethyl acetate with a catalytic amount of DMF (1.5 mL) was treated dropwise over about 45 minutes with oxalyl chloride (165 mL, 240 g, 1.9 mole). With the addition of the oxalyl chloride, vigorous gas evolution from the reaction mixture became evident; after the addition, the resulting mixture was stirred at ambient temperature thirty minutes. An additional portion of DMF (1.5 mL) was cautiously added and the mix stirred a further thirty minutes at ambient temperature. The virtually homogeneous reaction mixture was concentrated in vacuo on a rotary evaporator with the bath temperature held below 40° C. Heptanes were flashed off the residual solid (3×250 mL) to remove excess oxalyl chloride. This crude product, certainly containing residual amounts of heptanes, was used as is in the subsequent reaction in the scheme.

Preparation of INT-3: Crude acid chloride, INT-2, (crude product from oxalyl chloride reaction above; 1.50 mole) was suspended in 1.5 L of isopropyl ether then treated over about three minutes with a solution of t-butyl alcohol (300 mL, 3.2 mole) and N,N-dimethylaniline (300 mL, 2.4 mole). The stirred red mixture was heated to reflux over about 45 minutes then held there for two hours; the mixture was

15 stirred at ambient temperature overnight. The mixture was poured into solution prepared by diluting 250 mL concentrated hydrochloric acid to approximately 1.5 L with ice and water; this was followed by the addition of 1.5 L of THF and 1.5 L ethyl acetate. The mixture was agitated then the layers were separated; the organic layer was washed with 500 mL portions of 10% aqueous hydrochloric acid and water. The combined aqueous layers were extracted with a further 400 mL ethyl acetate. Finally the organic layers were combined, dried with anhydrous sodium sulfate (400 g), filtered and 20 concentrated in vacuo on a rotary evaporator; heptanes were flashed off (3×250 mL). The residual solid was dissolved in about 2.5 methanol and allowed to cool to ambient temperature overnight. The resulting semi-solid mass was mechanically broken up, then diluted with 500 mL methanol, stirred and vacuum filtered, pressed with rubber dam, washed with 250 mL cold methanol then finally air dried to afford INT-3 as a bright yellow solid (519 g, 87%), mp 66–68° C.

Preparation of INT-4: INT-3 (1007 g, 2.53 moles), 5% 25 palladium on carbon (75 g) and 7.5 L heptanes were charged into a hydrogenation apparatus. This reaction vessel was purged with nitrogen then pressurized with hydrogen gas to about 600 psi. The pressurized mixture was shaken and heated externally to 55–65° C.; heating and agitation continued for 24 h with the hydrogen pressure generally maintained near 600 psi by addition of more hydrogen gas. After 30 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880

solution was cooled, diluted with 3 L of aqueous ethyl alcohol (1:1 (v/v)) then chilled to allow solidification. The slurry stirred at reduced temperature for about 30 min then was filtered. The solids were pressed (rubber dam) at aspirator pressure, washed with 250 mL cold 1:1 aqueous ethyl alcohol then pulverized and air dried over 48 hours. INT-5 was obtained as a cream colored solid (917 g, 97%), mp 64–66° C.

Preparation of (crude) INT-6: A near solution of INT-5 (229.5g, 0.500mole) in 500 mL ethyl acetate was treated at once with activated manganese (IV) oxide (CAS 1313-13-9; 217.5 g, 2.50 mole). A mildly exothermic reaction ensued with the internal temperature eventually rising to 30–35° C. After one hour, the slurry was filtered through diatomaceous earth; the solids were wash with 250 mL ethyl acetate in portions. The filtrate was sequentially washed with 250 mL 10% hydrochloric acid and 250 mL water, then dried with sodium sulfate (250 g). The slurry was filtered, washing the solids with portions of ethyl acetate (ca. 250 mL total volume). The filtrate was treated with 2,6-lutidine (150 mL, 1.3 mole) then chilled to ca. 5° C. and treated over 30 min with a solution of phosgene in toluene (20% (w/w) 300 mL, 0.57 mole) such that the internal temperature remained at or below 18° C. This mix was stirred at reduced temperature for one hour. The reaction solution was decanted from the thick, pasty precipitate and filter through diatomaceous earth, the solids were washed with 250 mL ethyl acetate in portions. The combined filtrate was concentrated in vacuo, three portions of toluene (totaling 450 mL) were flashed off to afford crude INT-6.

Preparation of INT-7: The crude INT-6 (derived from the previous reaction sequence, ca. 0.500 mole) was dissolved in 500 mL pyridine then treated at once with methyl 2-mercaptop-4-thiazoleacetate (CAS 41714-97-0; 108.7 g, 0.575 mole). The resulting mixture was heated at 55–60° C. for ninety minutes. The reaction mixture was concentrated in vacuo with the residue partitioned between 1 L ethyl acetate/THF (1:1 (v/v)) and cold dilute acidic brine solution (150 mL concentrated hydrochloric acid plus 150 mL saturated brine diluted to 1 L with ice water). The organic layer was washed with 150 mL 10% hydrochloric acid. The combined aqueous washes were further extracted with 150 mL ethyl acetate. The combined organics were dried with sodium sulfate (400 g), filtered (washing with minimal ethyl acetate) and concentrated in vacuo. Heptanes were flashed off (450 mL in three portions) to provide a thick yellow-orange oil. The oil was triturated with 750 mL methyl alcohol overnight to allow thorough crystallization. The resultant slurry was chilled in an ice bath for an hour, filtered, washed with ice cold methyl alcohol (ca. 250 mL), pressed, then air dried to afford INT-7 as a bright yellow solid (245 g; 74%) mp 68–69° C.

Preparation of IRQ-1: A stirred slurry of INT-7 (240 g, 0.364 mole) in 350 mL toluene was treated over five minutes with 350 mL trifluoroacetic acid (4.54 mole). With the addition the reaction mixture's temperature initially fell slightly, then a mild exotherm was noted with the temperature finally reaching 30–35° C. The now homogenous mix was stirred at ambient temperature for two hours then concentrated in vacuo; portions of toluene (3×150 mL) were flashed off. The residue was dissolved in 750 mL propyl acetate; the solution was washed with two portions (250 mL) of 10% aqueous sodium acetate, then dried with sodium sulfate (250 g) and filtered, washing with minimal propyl acetate. The filtrate was diluted with of heptane (1 L), stirred to allow crystallization, then chilled in a ice bath for one hour. The cold slurry (ca. 5° C.) was filtered, the solids were washed with minimal cold 1:1 (v/v) propyl acetate/heptane, washed with low boiling ligroine (3×250 mL), then air dried to provide IRQ-1 as a bright yellow solid (202g, 92%), mp 82–83° C.

Preparation of Dispersion of IRQ-1: 1.0 g of IRQ-1 was dissolved in 2.0 g of N, N-Diethylauramide and 3.0 g of ethyl acetate with gentle heating. This solution was then brought to a temperature of 40° C. and then mixed with a solution containing 3.0 g of pig gelatin and 0.3 g of the sodium salt of triisopropylnaphthalene sulfonic acid dissolved in 40.7 g of distilled water. The resulting mixture was then passed through a colloid mill three times to produce a dispersion.

#### Photographic Example 1

Sample 101 (Invention): The following layers were coated in the following order onto a cellulose triacetate support subbed with gelatin using conventional coating techniques. In the composition of the layers, the coated amounts are given as g/m<sup>2</sup>. Laydowns of silver halide are given relative to silver. Emulsion sizes as determined by the disc centrifuge method are reported in diameter x thickness in microns. IRQ-1 was incorporated in the slow magenta recording layer in the form of a dispersion prepared as described above.

| 25 Layer 1: Antihalation Layer |      |
|--------------------------------|------|
| Black colloidal Silver         | 0.25 |
| UV Dye UV-1                    | 0.04 |
| UV Dye UV-2                    | 0.06 |
| Dispersed in Solvent S-1       | 0.04 |
| Gelatin                        | 2.15 |

| 35 Layer 2: Low speed Red Sensitive Layer                                                            |                  |
|------------------------------------------------------------------------------------------------------|------------------|
| Silver Iodobromide emulsion                                                                          | 0.36 (as silver) |
| 1.06 $\mu$ m by 0.092 $\mu$ m, 4% bulk iodide emulsion spectrally sensitized with dyes SD-0 and SD-1 |                  |
| Fine Grain Silver Bromide                                                                            | 0.05 (as silver) |
| 0.055 $\mu$ m equivalent spherical diameter                                                          |                  |
| Cyan Coupler C-1                                                                                     | 0.10             |
| Dispersed in Solvent S-3                                                                             | 0.05             |
| Gelatin                                                                                              | 1.07             |

| 45 Layer 3: Medium Speed Red Sensitive Layer                                                 |                  |
|----------------------------------------------------------------------------------------------|------------------|
| Silver Iodobromide Emulsion                                                                  | 0.43 (as silver) |
| 0.85 $\mu$ m by 0.090 $\mu$ m, 4% bulk iodide, spectrally sensitized with dyes SD-0 and SD-1 |                  |
| Fine Grain Silver Bromide                                                                    | 0.06 (as silver) |
| 0.055 $\mu$ m equivalent spherical diameter                                                  |                  |
| Cyan Coupler C-1                                                                             | 0.53             |
| Dispersed in Solvent S-3                                                                     | 0.20             |
| Gelatin                                                                                      | 0.94             |

| 55 Layer 4: High Speed Red Sensitive Layer                                                                  |                  |
|-------------------------------------------------------------------------------------------------------------|------------------|
| Silver Iodobromide Emulsion                                                                                 | 0.49 (as silver) |
| 1.18 $\mu$ m by 0.111 $\mu$ m, 3% bulk iodide, spectrally sensitized with dyes SD-0 and SD-1                |                  |
| Fine Grain Silver Iodobromide                                                                               | 0.03             |
| 0.15 $\mu$ m equivalent spherical diameter, 4.8% bulk iodide, spectrally sensitized with dyes SD-0 and SD-1 |                  |
| Fine Grain Silver Bromide                                                                                   | 0.065            |

-continued

|                                                                                                                  |                  |
|------------------------------------------------------------------------------------------------------------------|------------------|
| Layer 4: High Speed Red Sensitive Layer                                                                          |                  |
| 0.055 $\mu\text{m}$ equivalent spherical diameter                                                                | 5                |
| Cyan Coupler C-1                                                                                                 | 0.77             |
| Dispersed in Solvent S-3                                                                                         | 0.385            |
| Gelatin                                                                                                          | 1.30             |
|                                                                                                                  | 10               |
| Layer 5: First Interlayer                                                                                        |                  |
| Filter Dye FD-1                                                                                                  | 15               |
| SCV-1                                                                                                            | 0.16             |
| Dispersed in Solvent S-3                                                                                         | 0.32             |
| Gelatin                                                                                                          | 0.81             |
|                                                                                                                  | 20               |
| Layer 6: Second Interlayer                                                                                       |                  |
| Carey Lea Silver                                                                                                 | 25               |
| Gelatin                                                                                                          | 0.81             |
|                                                                                                                  | 30               |
| Layer 7: Low Speed Green Sensitive Layer                                                                         |                  |
| Silver Iodobromide Emulsion                                                                                      | 35               |
| 0.62 $\mu\text{m}$ by 0.064 $\mu\text{m}$ , 4% bulk iodide, spectrally sensitized with dyes SD-4 and SD-5        | 0.45 (as silver) |
| Fine Grain Silver Bromide                                                                                        | 0.10 (as silver) |
| 0.055 $\mu\text{m}$ equivalent spherical diameter                                                                | 35               |
| Magenta Coupler M-1                                                                                              | 0.17             |
| Magenta Coupler M-2                                                                                              | 0.07             |
| co-dispersed in Solvent S-2                                                                                      | 0.12             |
| IRQ-1                                                                                                            | 0.014            |
| Dispersed with solvent S-4                                                                                       | 0.028            |
| Gelatin                                                                                                          | 1.10             |
|                                                                                                                  | 40               |
| Layer 8: Medium Speed Green Sensitive Layer                                                                      |                  |
| Silver Iodobromide Emulsion                                                                                      | 45               |
| 0.96 $\mu\text{m}$ by 0.065 $\mu\text{m}$ , 3% bulk iodide, spectrally sensitized with dyes SD-4 and SD-5        | 0.37 (as silver) |
| Fine Grain Silver Bromide                                                                                        | 0.05 (as silver) |
| 0.055 $\mu\text{m}$ equivalent spherical diameter                                                                | 45               |
| Magenta Coupler M-1                                                                                              | 0.33             |
| Magenta Coupler M-2                                                                                              | 0.14             |
| Co-dispersed in Solvent S-2                                                                                      | 0.235            |
| Gelatin                                                                                                          | 0.87             |
|                                                                                                                  | 50               |
| Layer 9: High Speed Green Sensitive Layer                                                                        |                  |
| Silver Iodobromide Emulsion                                                                                      | 55               |
| 1.18 $\mu\text{m}$ by 0.111 $\mu\text{m}$ , 3% bulk iodide, spectrally sensitized with dyes SD-4 and SD-5        | 0.47 (as silver) |
| Fine Grain Silver Iodobromide emulsion                                                                           | 60               |
| 0.15 $\mu\text{m}$ equivalent spherical diameter, 4.8% bulk iodide spectrally sensitized with dyes SD-4 and SD-5 | 0.04 (as silver) |
| Magenta Coupler M-1                                                                                              | 0.62             |
| Magenta Coupler M-2                                                                                              | 0.27             |

-continued

|                                                                                                           |                  |
|-----------------------------------------------------------------------------------------------------------|------------------|
| Layer 9: High Speed Green Sensitive Layer                                                                 |                  |
| Co-dispersed in Solvent S-2                                                                               | 5                |
| Gelatin                                                                                                   | 0.445            |
|                                                                                                           | 1.53             |
| Layer 10: Third Interlayer                                                                                |                  |
| Gelatin                                                                                                   | 10               |
|                                                                                                           | 0.61             |
| Layer 11: Fourth Interlayer                                                                               |                  |
| Carey Lea Silver                                                                                          | 15               |
| SCV-1                                                                                                     | 0.07             |
| Dispersed in solvent S-3                                                                                  | 0.11             |
| Gelatin                                                                                                   | 0.22             |
|                                                                                                           | 20               |
| Layer 12: Low Speed Blue Sensitive Layer                                                                  |                  |
| Silver Iodobromide Emulsion                                                                               | 25               |
| 1.47 $\mu\text{m}$ by 0.135 $\mu\text{m}$ , 3% bulk iodide, spectrally sensitized with dyes SD-6 and SD-7 | 0.27 (as silver) |
| Silver Iodobromide Emulsion                                                                               | 30               |
| 1.07 $\mu\text{m}$ by 0.139 $\mu\text{m}$ , 3% bulk iodide, spectrally sensitized with dyes SD-6 and SD-7 | 0.27 (as silver) |
| Fine Grain Silver Bromide                                                                                 | 35               |
| 0.055 $\mu\text{m}$ equivalent spherical diameter                                                         | 0.07 (as silver) |
| Yellow Coupler YEL-1                                                                                      | 1.27             |
| Dispersed in Solvent S-3                                                                                  | 0.42             |
| Gelatin                                                                                                   | 1.89             |
|                                                                                                           | 40               |
| Layer 13: High Speed Blue Sensitive Layer                                                                 |                  |
| Silver Iodobromide Emulsion                                                                               | 45               |
| 2.59 $\mu\text{m}$ by 0.147 $\mu\text{m}$ , 2% bulk iodide, spectrally sensitized with dyes SD-6 and SD-7 | 0.22 (as silver) |
| Silver Iodobromide Emulsion                                                                               | 50               |
| 1.86 $\mu\text{m}$ by 0.133 $\mu\text{m}$ , 2% bulk iodide, spectrally sensitized with dyes SD-6 and SD-7 | 0.22 (as silver) |
| Yellow Coupler YEL-1                                                                                      | 0.85             |
| Dispersed in Solvent S-3                                                                                  | 0.28             |
| Gelatin                                                                                                   | 1.13             |
|                                                                                                           | 55               |
| Layer 14: Fifth Interlayer                                                                                |                  |
| SCV-1                                                                                                     | 60               |
| Dispersed in solvent S-3                                                                                  | 0.16             |
| Gelatin                                                                                                   | 0.32             |
|                                                                                                           | 65               |
| Layer 15: First Overcoat                                                                                  |                  |
| Silver iodobromide emulsion                                                                               | 65               |
| 0.58 $\mu\text{m}$ by 0.062 $\mu\text{m}$ , 4% bulk iodide, spectrally sensitized with dyes SD-0 and SD-1 | 0.09 (as silver) |

-continued

| Layer 15: First Overcoat                          |                  | 5  | Layer 17: Third Overcoat                                                                                               |                    |
|---------------------------------------------------|------------------|----|------------------------------------------------------------------------------------------------------------------------|--------------------|
| Fine Grain Silver Bromide                         | 0.43 (as silver) |    | Matte                                                                                                                  | 0.02               |
| 0.055 $\mu\text{m}$ equivalent spherical diameter |                  |    | 1.7 $\mu\text{m}$ spherical diameter                                                                                   |                    |
| Gelatin                                           | 0.81             | 10 | Hardener H-1                                                                                                           | 1.38% of total gel |
|                                                   |                  |    | Gelatin                                                                                                                | 0.97               |
|                                                   |                  |    |                                                                                                                        |                    |
| Layer 16: Second Overcoat                         |                  | 15 | The components employed for the preparation of light-sensitive materials not already identified above are shown below: |                    |
| UV Dye UV-4                                       | 0.41             |    |                                                                                                                        |                    |
| UV Dye UV-1                                       | 0.09             |    |                                                                                                                        |                    |
| Dispersed in Latex L-1                            | 0.45             |    |                                                                                                                        |                    |
| Gelatin                                           | 1.40             |    |                                                                                                                        |                    |

SCV-1:



C-1:



M-1:



M-2:



YEL-1:



FD-1:



35

36

-continued

SD-0:



SD-1:



SD-4:



SD-5:



SD-6:



SD-7:



UV-1:



UV-2:



UV-4:



L-1:



## Hardener H-1:

1,1'-[methylenebis(sulfonyl)]bis-ethene

## Solvent S-1

1,4-Cyclohexylenedimethylene bis(2-ethylhexanoate)

## Solvent S-2

Phosphoric Acid, tris(methylphenyl) ester

## Solvent S-3

1,2-benzenedicarboxylic acid, dibutyl ester

## Solvent S-4

N,N-Diethylauramide

Samples 102 to 108 were prepared in a similar fashion to Sample 101, except that IRQ-1 was replaced with the inhibitors as indicated below in the mounts shown in g/m<sup>2</sup>.

Sample 102 (Invention): IRQ-2 at 0.013

Sample 103 (Invention): IRQ-3 at 0.013

Sample 104 (Invention): IRQ-4 at 0.013

Sample 105 (Invention): IRQ-5 at 0.013

Sample 106 (Invention): IRQ-6 at 0.014

Sample 107 (Comparative example): CMMT at 0.001

Sample 108 (Comparative example): no addenda

The samples were evaluated to determine the impact of the IRQ compounds on color modification via IIE effects, image sharpness, and photographic speed. Standard stepped sensitometric exposures to daylight-balanced white light were employed to measure speed differences between the coatings; speed differences measured at density equal to 0.5 are tabulated in Table 1 in CR units with 1.0 CR unit being equal to a difference of 0.01 log exposure relative to Sample 108. IIE effects were determined by exposing film to a red step exposure as well as to a uniform green flash exposure. The change in green density (at a flash level near D=1.0) with increasing red exposure was then measured. Increasing differences in green density change indicated higher levels of IIE; these data are also tabulated in Table 1.

The sharpness of images recorded in each of the three color records of the test Samples was determined by measuring the acutance using standard power spectrum methods (represented as 8X loupe DMT's as described in *J. Soc. Photogr. Technol. Japan*, Vol. 62, No. 2, 1999, page 112), with higher acutance responses correlating with increased image sharpness. These data are summarized in Table 1. The speed and acutance data are presented as a difference from Sample 108 which contained no addenda. After exposing as described, all test Samples were developed employing standard Kodak E-6 color reversal processing solutions.

TABLE 1

| Sam-<br>ple | In-<br>hibitor | Red on<br>Green   |     |       | IIE<br>(D =<br>1.0) | Δ Acutance<br>8X loupe DMT |       |      |
|-------------|----------------|-------------------|-----|-------|---------------------|----------------------------|-------|------|
|             |                | Δ Speed (D = 0.5) | Red | Green |                     | Red                        | Green | Blue |
| 101         | IRQ-1          | -17               | -12 | -10   | 0.70                | 2.4                        | 2.8   | 2.6  |
| 102         | IRQ-2          | -15               | -14 | -07   | 0.57                | 1.3                        | 1.9   | 1.7  |
| 103         | IRQ-3          | -02               | -05 | -01   | 0.49                | 0                          | 1.1   | 0.7  |
| 104         | IRQ-4          | -10               | -09 | -04   | 0.48                | 1.0                        | 1.6   | 1.4  |
| 105         | IRQ-5          | -28               | -21 | -14   | 0.66                | 2.9                        | 2.5   | 2.6  |
| 106         | IRQ-6          | -14               | -17 | -08   | 0.59                | 2.0                        | 3.2   | 2.8  |
| 107         | CMMT           | -31               | -21 | -14   | 0.74                | 2.5                        | 1.9   | 2.1  |
| 108         | None           | 0                 | 0   | 0     | 0.41                | 0                          | 0     | 0    |
|             | (Check)        |                   |     |       |                     |                            |       |      |

From the data in Table 1 it is clear that the IRQ compounds of the invention greatly enhance the IIE and sharpness of the films relative to the comparative example Sample 108 which contains no addenda. More over, the IRQ com-

pounds of the invention clearly provide such beneficial increases in IIE and sharpness with smaller attendant losses in photographic speed relative to the comparative example Sample 107 which contained CMMT.

To assess the relative merit of the IRQ compounds relative to the standard use of CMMT, a ratio of acutance improvement versus speed penalty was calculated for each color record ( $\Delta$ Acutance $\times$ 100/ $\Delta$ Speed). The higher this ratio the more acutance is obtain per unit speed loss; these ratios are arrayed in Table 2. It is clear from these data that the IRQ's afford improvements in image sharpness with a smaller speed disadvantage than obtained with CMMT. In virtually every color record where acutance improvements were noted, the IRQ compounds afforded a lower speed penalty.

TABLE 2

| Sample | Inhibitor | Δ Acutance $\times$ 100/ $\Delta$ Speed |       |      |
|--------|-----------|-----------------------------------------|-------|------|
|        |           | Red                                     | Green | Blue |
| 101    | IRQ-1     | 14.1                                    | 23.3  | 12.0 |
| 102    | IRQ-2     | 8.6                                     | 13.6  | 5.7  |
| 103    | IRQ-3     | 0                                       | 22.0  | 10.0 |
| 104    | IRQ-4     | 10.0                                    | 17.7  | 17.5 |
| 105    | IRQ-5     | 10.3                                    | 11.9  | 10.7 |
| 106    | IRQ-6     | 14.3                                    | 18.8  | 21.2 |
| 107    | CMMT      | 8.1                                     | 9.0   | 6.4  |

These data indicate the exceptional utility of the IRQ compounds in providing both color improving IIE's as well as dramatic improvements in image acutance. These improvements in photographic acutance, often surpassing those available from CMMT, were obtained with substantially smaller speed penalties than those encountered with the current commercial technology.

## Photographic Example 2

For a reversal format, the blocked IRQ compounds of formula F-1 may be coated with appropriately sensitized silver iodobromide emulsions on a support bearing the following layers from top to bottom:

- (1) one or more overcoat layers;
- (2) a nonsensitized silver halide containing layer;
- (3) a triple-coat yellow layer pack with a fast yellow layer containing "Coupler 1": Benzoic acid, 4-(1-((2-chloro-5-((dodecylsulfonyl)amino)phenyl)amino)carbonyl)-3,3-dimethyl-2-oxobutoxy-, 1-methylethyl ester; a mid yellow layer containing Coupler 1 and "Coupler 2": Benzoic acid, 4-chloro-3-[[2-[4-ethoxy-2,5-dioxo-3-(phenylmethyl)-1-imidazolidinyl]-4,4-dimethyl-1,3-dioxopentyl]amino]-, dodecylester; and a slow yellow layer also containing Coupler 2;
- (4) an interlayer;
- (5) a layer of fine-grained silver;
- (6) an interlayer;
- (7) a triple-coated magenta pack with a fast and mid magenta layer containing "Coupler 3": 2-Propenoic acid, butyl ester, polymer with N-[1-(2,5-dichlorophenyl)-4,5-dihydro-5-oxo-1H-pyrazol-3-yl]-2-methyl-2-propenamide; "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl); and "Coupler 5": Benzamide, 3-((2,4-bis(1,1-dimethylpropyl)phenoxy)-acetyl)amino)-N-(4,5-dihydro-5-oxo-1-2,4,6-trichlorophenyl)-1H-pyrazol-3-yl); and containing the stabilizer 1,1'-Spirobi(1H-indene), 2,2',3,3'-

39

tetrahydro-3,3,3',3'-tetramethyl-5,5',6,6'-tetrapropoxy-; and in the slow magenta layer Couplers 4 and 5 with the same stabilizer;

- (8) one or more interlayers possibly including fine-grained nonsensitized silver halide;
- (9) a triple-coated cyan pack with a fast cyan layer containing "Coupler 6": Tetradecanamide, 2-(2-cyanophenoxy)-N-(4-((2,2,3,3,4,4,4-heptafluoro-1-oxobutyl)amino)-3-hydroxyphenyl)-; a mid cyan containing "Coupler 7": Butanamide, N-(4-((2,4-bis(1,1-dimethylpropyl)phenoxy)-1-oxobutyl)amino)-2-hydroxyphenyl)-2,2,3,3,4,4,4-heptafluoro- and "Coupler 8": Hexanamide, 2-(2,4-bis(1,1-dimethylpropyl)-phenoxy)-N-(4-((2,2,3,3,4,4,4-heptafluoro-1-oxobutyl)amino)-3-hydroxyphenyl)-; and a slow cyan layer containing Couplers 6, 7, and 8;
- (10) one or more interlayers possibly including fine-grained nonsensitized silver halide; and
- (11) an antihalation layer.

The invention has been described in detail with particular reference to certain preferred embodiments thereof, but it will be understood that variations and modifications can be effected within the spirit and scope of the invention.

We claim:

1. A multilayer color reversal photographic element comprising a support and at least two photographic silver halide emulsion layers and a compound of the formula F-1:



F-1 30  
35

wherein A, B, C, and D are independently substituted or unsubstituted aliphatic, alicyclic, aromatic or heterocyclic substituents, which may where structurally possible together form a ring or rings; where at least one of A, B, C, and D is of the formula F-2:



F-2 45  
50

wherein R<sup>1</sup> and R<sup>2</sup> are independently either hydrogen or substituted or unsubstituted aliphatic, alicyclic, aromatic or heterocyclic substituents, which may where structurally possible form a ring with other substituents; R<sup>3</sup> is a substituted or unsubstituted aliphatic, alicyclic, aromatic or heterocyclic substituent which may where structurally possible form a ring with other substituents, L is a bivalent linking or linking group attached to the carbonyl moiety via a heteroatom; n varies from 0-2; and INH is a silver development inhibitor attached either to an L or the carbonyl moiety via a heteroatom.

2. An element according to claim 1, wherein R<sup>1</sup> and R<sup>2</sup> are hydrogen or lower alkyl groups of from 1 to 4 carbon atoms and R<sup>3</sup> is an alkyl group of from 1-12 carbon atoms for at least one F-2 substituent of the F-1 compound.

40

3. An element according to claim 2, wherein R<sup>3</sup> is a primary alkyl group.

5 4. An element according to claim 2, wherein the A, B, C and D substituents which are not of structure F-2 are independently alkyl or aryl groups of from 1-20 carbon atoms, or two of such groups combine together to form a non-aromatic ring.

10 5. An element according to claim 1, wherein NH comprises a mercaptotetrazole, selenotetrazole, mercaptobenzothiazole, selenobenzothiazole, mercaptobenzoxazole, selenobenzoxazole, benzotriazole, and benzodiazole, mercaptoxadiazole, mercaptothiadiazole, or mercaptothiazole compound.

15 6. An element according to claim 1, wherein NH is of the formula:



INH-1



INH-2



INH-3



INH-4



INH-5



INH-6



INH-7



INH-8



INH-9



41

-continued



where R<sup>7</sup> and R<sup>8</sup> are individually hydrogen or a substituted or unsubstituted alkyl or phenyl group, and R<sup>9</sup> and R<sup>10</sup> are individually hydrogen or one or more halogen, alkyl, carboxyl, carboxy esters, —NHCOOCH<sub>3</sub>, —SO<sub>2</sub>OCH<sub>3</sub>, —OCH<sub>2</sub>CH<sub>2</sub>SO<sub>2</sub>CH<sub>3</sub>, —OC(O)OCH<sub>2</sub>CH<sub>3</sub>, —NHC(O)C(O)OCH<sub>3</sub> or nitro groups.

7. An element according to claim 1, wherein the compound of formula F-1 comprises a solubilization group having a pKa less than 10.

8. An element according to claim 7, wherein the solubilization group comprises a carboxylic acid, carboxylate salt, sulfonic acid, sulfonic acid, cyanamide, sulfonamide, hydroxamic acid, thiol, or thiolate.

9. An element according to claim 1, wherein INH is of the structure:



where R<sub>i</sub> is hydrogen or alkyl group of from 1-4 carbon atoms.

42

INH-10

10. An element according to claim 1, wherein only one of the A, B, C, D substituents is of the structure F-2, and the meta and para positioned substituents relative to the F-2 substituent form a non-aromatic carbocyclic ring fused with the quinone ring.

11. An element according to claim 10, wherein the ortho positioned substituent relative to the F-2 substituent is a primary, secondary, or tertiary alkyl group, and the R<sup>3</sup> group of the F-2 substituent is a primary alkyl group.

12. An element according to claim 1, wherein at least two of the A, B, C, D substituents are of the structure F-2.

13. An element according to claim 12, wherein the two F-2 substituents are positioned para with respect to each other.

14. An element according to claim 1, where any remaining A, B, C, and D substituents which are not of structure F-2 are primary, secondary, or tertiary alkyl groups.

15. A process for developing a photographic element according to claim 1 after imagewise exposure, comprising subjecting the exposed element to a color reversal process comprising a first black and white development step which develops a silver image in negative exposed areas, a reversal fogging step, and then development with a chromogenic developer to form a positive color image.

16. An element according to claim 1, wherein n=0.

17. An element according to claim 4, wherein n=0.

18. An element according to claim 9, wherein n=0.

19. An element according to claim 10, wherein n=0.

20. An element according to claim 7, wherein the solubilization group comprises a carboxylic acid moiety.

\* \* \* \* \*

UNITED STATES PATENT AND TRADEMARK OFFICE  
**CERTIFICATE OF CORRECTION**

PATENT NO. : 6,521,400 B1  
DATED : February 18, 2003  
INVENTOR(S) : Dannhauser et al.

Page 1 of 1

It is certified that error appears in the above-identified patent and that said Letters Patent is hereby corrected as shown below:

Column 40,  
Lines 11 and 19, change "NH" to -- INH --

Signed and Sealed this

Thirtieth Day of November, 2004



JON W. DUDAS  
*Director of the United States Patent and Trademark Office*